

1

3,185,646

# **CORROSION INHIBITED LUBRICANTS**

**CORROSION INHIBITED LUBRICANTS**  
Robert G. Anderson, Novato, and Yngve G. Hendrickson,  
El Cerrito, Calif., assignors to California Research  
Corporation, San Francisco, Calif., a corporation of  
Delaware  
No Drawing. Filed Sept. 28, 1962, Ser. No. 227,052  
5 Claims. (Cl. 252—46.7)

This invention pertains to lubricating oil compositions having incorporated therein metal-free detergents. These particular detergents are also effective as corrosion inhibitors.

Present day internal combustion engines operate at high speeds and high compression ratios. When used in the so-called City stop-and-go driving, which includes the greater part of the driving conditions for a large percentage of today's automobiles, the internal combustion engines do not reach the most efficient operating temperature. Under City driving conditions, large amounts of partial oxidation products are formed, and reach the crankcase of the engine by blowing past the piston rings. This phenomenon is noticed more in engines having greater wear during the break-in period. Most of the partial oxidation products are oil-insoluble, tending to form deposits on the various operating parts of the engine, such as the pistons, piston rings, etc. For the purpose of preventing the deposition of these products on the various engine parts, and to reduce break-in wear, it is necessary to incorporate detergents and wear-reducing agents in the lubricating oil compositions, thus keeping these polymeric products dispersed in a condition unfavorable for deposition on metals.

A great number of the detergents which are added to crankcase oils to reduce this formation of sludges and varnishes are metal organic compounds, particularly those compounds wherein the metal is linked to an organic group through an oxygen atom. Although these metal-containing organic compounds have some effectiveness as detergents for dispersing the precursors of the deposits within the oil itself rather than permitting them to form as deposits on the engine parts, they have the disadvantage of forming ash deposits in the engine. These ash deposits lower engine performance by fouling spark plugs and valves, and contributing to pre-ignition.

It is a particular object of this invention to provide lubricating oil compositions having incorporated therein metal-free detergents which are also effective as corrosion inhibitors. Thus, these new additives disperse the undesirable polymeric products which are formed, and also inhibit corrosion to metal wearing surfaces.

Therefore, in accordance with this invention, it has been found that lubricating oil compositions particularly useful for heavy duty service are obtained by incorporating therein a product obtained by (1) reacting an alkenyl succinic anhydride with phosphorus pentasulfide followed by (2) reacting the product of (1) with a polyalkylene polyamine.

By the use of lubricating oil compositions containing the reaction products described herein, diesel and gasoline engine parts remain remarkably free of deposits and varnish, even under severe operating conditions. In addition these lubricating oils reduce break-in-wear.

The alkenyl succinic anhydride reactants are of the formula

2

wherein R is a hydrocarbon radical having from 30 to 200 carbon atoms therein, preferably from 50 to 200 carbon atoms.

Examples of alkenyl radicals include propylene polymers containing from 30 to 200 carbon atoms, and polymers of mixtures of 1-butene and isobutene having from 30 to 200 carbon atoms.

The polyalkylene polyamines, which contribute the imide nitrogen and the basic nitrogen atoms of the reaction products herein, are derived from polymers of ethylene or propylene, such as polyethylene polyamine, and polypropylene polyamines. Such polyalkylene polyamines may be represented by the formula



wherein the R represents the divalent radical ethylene or propylene, and x is a number having a value from 1 to 10 or more. Examples of these polyalkylene polyamines include diethylene triamine, triethylene tetramine, tetraethylene pentamine, pentaethylene hexamine, di-propylene triamine, dipropylene tetramine, tetrapropylene pentamine, pentapropylene hexamine, di-(trimethylene) triamine, tri(trimethylene), tetramine, tetra-(trimethylene) petamine and penta-(trimethylene hexamine).

Other polyalkylene polyamines can be exemplified by the aminoalkyl piperazines, for example,  $\beta$  aminoethyl piperazine.

The mol ratio of phosphorus pentasulfide to succinic anhydride can vary from 5:1 to .5:1; preferably, 1.5:1 to 3:1.

With regard to the polyalkylene polyamine, the molar ratio of polyalkylene polyamine to anhydride can range from 0.5 to 1.5, preferably 0.8 to 1.2.

In the reaction herein between the anhydride and the  $P_2S_5$ , the reaction temperature can vary from 100° F. to 450° F., preferably from 250° F. to 350° F.

In the reaction between the  $P_2S_5$  anhydride product and polyamine, the reaction temperature is from 250° F. to about 450° F., preferably 280° F. to 350° F.

Lubricating oils which can be used as base oils to form lubricating oils suitable for the above-mentioned applications.

lubricating oil compositions of the above-described additives include a wide variety of lubricating oils, such as naphthenic base, paraffin base, and mixed base lubricating oils, other hydrocarbon lubricants, e.g., lubricating oils derived from mineral oil, vegetable oil, animal oil, and the like.

derived from coal products, and synthetic oils, e.g., alkylene polymers (such as polymers of propylene, butylene, etc., and the mixtures thereof), alkylene oxide-type polymers (e.g., propylene oxide polymers) and derivatives, including alkylene oxide polymers prepared by polymerizing the alkylene oxide in the presence of water or alcohols, e.g., ethyl alcohol, dicarboxylic acid esters (such as those which are prepared by esterifying such dicarboxylic acids as adipic acid, azelaic acid, suberic acid, sebacic

acid, alkenyl succinic acid, fumaric acid, maleic acid, etc., with alcohols such as butyl alcohol, hexyl alcohol, 2-ethyl hexyl alcohol, dodecyl alcohol, etc.), liquid esters of acids of phosphorus, alkyl benzenes, (e.g., monoalkyl benzene such as dodecyl benzene, tetradecyl benzene, etc.).

and dialkyl benzenes (e.g., n-nonyl 2-ethyl hexyl benzene); polyphenyls (e.g., biphenyls and terphenyls), alkyl biphenyl esters, compounds of silicon (e.g., tetraethyl silicate, tetraisopropyl silicates, tetra(4-methyl-2-tetraeth-

siloxane, poly(methyl-phenyl-phenyl), poly(methyl-phenyl-phenyl-phenyl) silicate, hexyl (4-methyl-2-pentoxy) disiloxane, poly(methyl) siloxane, poly(methyl-phenyl) siloxane, etc. Synthetic oils of the alkylene oxide-type polymers which may be used include those exemplified by the alkylene

The products described herein can be used in oils in amounts of .1% to 40% by weight, preferably 0.1% to 15%, by weight; more preferably, 1% to 10%.



reaction product useful herein as corrosion inhibitors and detergents.

EXAMPLE I

A mixture of 94 grams of phosphorus pentasulfide, 500 grams of polyisobutetyl succinic anhydride, wherein the polyisobutetyl radical contained approximately 66 carbon atoms, and 500 grams of xylene was heated at reflux temperatures for a period of 12 hours. The xylene was distilled off under reduced pressure. For convenience the product is called Product A.

250 grams of Product A cooled to 200° F. was added dropwise to a flask containing 16.6 grams of tetraethylene pentamine heated to 200 F. The reaction mixture was blanketed with nitrogen. After all of Product A had been added, the mixture was heated to 310° F. The reaction mixture was heated at this temperature for 0.25 hour at an absolute pressure of about 200 mm. Hg followed by 0.75 hour at an absolute pressure of 5 mm. Hg.

The remaining reaction product contained:

|            | Weight percent |
|------------|----------------|
| Phosphorus | 3.21           |
| Sulfur     | 5.94           |
| Nitrogen   | 2.23           |

Table I hereinbelow presents further data on the effectiveness of the reaction products described herein as lubrication oil additives. The data of Table I were obtained after 60 hours of operating under the severe conditions of a Caterpillar 1-H engine test used to qualify oils under the 2104 B procedure. This Military specification procedure is so severe that the engine will not even operate with a base oil uncompounded. Even a base oil with the normal commercial additives under this procedure does not provide sufficient lubrication; that is, the engine itself eventually sticks.

The base oil used in obtaining data for Table I consisted of a California paraffinic base oil having a viscosity of 500 SSU at 100° F., and having incorporated therein 15 mM./kg. (i.e., 15 millimols of metal per kilogram of the finished lubricating oil composition) of a basic sulfurized calcium phenate, and 12 mM./kg. of a zinc dialkyl dithiophosphate.

The "PD Nos." refer to the piston discoloration rating. After the engine test, the three piston lands are examined visually. To a piston land which is completely black is assigned a PD No. of 800; to one which is completely clean, a PD No. 0; to those intermediate between those completely black and completely clean are assigned PD Nos. intermediate in proportion to the extent and degree of darkening.

The "GD Nos." refer to the percentage deposit in the

piston ring grooves; that is, a 0 evaluation being a clean groove, and a 100 evaluation being a groove full of deposits.

The mol ratio of the phosphorus pentasulfide to the anhydride was 2:1.

Table I

| 10                                      | Composition       | PD No. | GD No. | Break-in-Wear, mgs. loss |
|-----------------------------------------|-------------------|--------|--------|--------------------------|
| 1. Base Oil                             |                   |        |        |                          |
| 2. Base oil+4% wt. Product of Example I | 450, 235, 220, 15 | 10     |        | 628                      |

15 We claim:

1. A lubricating oil composition comprising a major proportion of an oil of lubricating viscosity and from 0.1% to 40%, by weight, of a product obtained by reacting (1) an alkenyl succinic anhydride having from 30 to 20 200 carbon atoms in the alkenyl radical with phosphorus pentasulfide at temperatures in the range of 100° F. to 450° F. wherein the phosphorus pentasulfide-anhydride mol ratio is from 5:1 to 0.5:1 followed by (2) reacting the product of (1) with a polyalkylene polyamine at temperatures from 250° F. to 450° F. wherein the mol ratio of said polyamine to said anhydride is from 0.5:1 to 1:1, said polyalkylene polyamine being of the formula



30 wherein R is selected from the group consisting of ethylene and propylene and x is a number from 1 to 10.

2. The lubricating oil composition of claim 1 wherein said product is present in amounts from 0.1 to 15% by weight.

35 3. The lubricating oil composition of claim 2 wherein said phosphorus pentasulfide-anhydride mole ratio is from 3:1 to 1.5:1.

4. The lubricating oil composition of claim 3 wherein said phosphorus pentasulfide-anhydride is reacted with 40 said polyalkylene polyamine at temperatures from 280° F. to 350° F.

5. The lubricating oil composition of claim 4 wherein said polyalkylene polyamine is tetraethylene pentamine.

45 References Cited by the Examiner

UNITED STATES PATENTS

|           |       |                 |          |
|-----------|-------|-----------------|----------|
| 2,733,235 | 1/56  | Cross et al.    | 252—32.7 |
| 2,773,862 | 12/56 | Musselman       | 252—32.7 |
| 3,018,247 | 1/62  | Anderson et al. | 252—32.7 |

50 DANIEL E. WYMAN, Primary Examiner.

UNITED STATES PATENT OFFICE  
CERTIFICATE OF CORRECTION

Patent No. 3,185,646

May 25, 1965

Robert G. Anderson et al.

It is hereby certified that error appears in the above numbered patent requiring correction and that the said Letters Patent should read as corrected below.

Column 2, lines 23 and 24, for "di-trimethylene)" read -- di(trimethylene) --; line 24, after "tri(trimethylene)" strike out the comma; lines 24 and 25, for "tetra-(trimethylene) petamine and penta-(trimethylene hexamine" read -- tetra-(trimethylene) pentamine and penta-(trimethylene) hexamine --; line 41, for "Lubricatin" read -- Lubricating --; line 43, for "vairety" read -- variety --; same column 2, line 62, for "esters" read -- ethers --; column 3, line 13, for "200 F." read -- 200° F. --; lines 26 and 27, for "lubrication" read -- lubricating --; same column 3, line 34, for "proivde" read -- provide --.

Signed and sealed this 26th day of October 1965.

(SEAL)

Attest:

ERNEST W. SWIDER  
Attesting Officer

EDWARD J. BRENNER  
Commissioner of Patents

UNITED STATES PATENT OFFICE  
CERTIFICATE OF CORRECTION

Patent No. 3,185,646

May 25, 1965

Robert G. Anderson et al.

It is hereby certified that error appears in the above numbered patent requiring correction and that the said Letters Patent should read as corrected below.

Column 2, lines 23 and 24, for "di-trimethylene)" read -- di(trimethylene) --; line 24, after "tri(trimethylene)" strike out the comma; lines 24 and 25, for "tetra-(trimethylene) petamin and penta-(trimethylene hexamine" read -- tetra-(trimethylene) pentamine and penta-(trimethylene) hexamine --; line 41, for "Lubricatin" read -- Lubricating --; line 43, for "vairety" read -- variety --; same column 2, line 62, for "esters" read -- ethers --; column 3, line 13, for "200 F." read -- 200° F. --; lines 26 and 27, for "lubrication" read -- lubricating --; same column 3, line 34, for "proivde" read -- provide --.

Signed and sealed this 26th day of October 1965.

(SEAL)

Attest:

ERNEST W. SWIDER

Attesting Officer

EDWARD J. BRENNER

Commissioner of Patents